

## UNITED STATES PATENT OFFICE

2,152,532

BLEACHING WITH ORGANIC BLEACHING  
AGENT

Paul J. Carlisle, Niagara Falls, N. Y., assignor to  
E. I. du Pont de Nemours & Company, Wil-  
mington, Del., a corporation of Delaware

No Drawing. Application December 30, 1937,  
Serial No. 182,625

3 Claims. (Cl. 8—108)

This invention relates to a novel and superior bleaching agent. More specifically, it relates to the use of the stable organic hypochlorite, tertiary butyl hypochlorite, having the formula 5  $(CH_3)_3C.OCl$  as a bleaching agent for bleaching material such as cotton, wool, and other textile fibers and fabrics generally, foodstuffs such as fruit and butter, and fatty and waxy materials such as wool fat, various oils and sulphonated 10 oils, and various waxes.

The alkyl hypochlorites including tertiary butyl hypochlorite have already been prepared. As the lower members of the series were found to be relatively explosive, and all of these hypochlorites 15 generally unstable, no attempt at commercial utilization of the compounds has been made. Recent research has now indicated that the tertiary alkyl hypochlorites are more stable than the primary and secondary hypochlorites. 20 Among the tertiary alkyl hypochlorites, I have found that tertiary butyl hypochlorite,  $(CH_3)_3C.OCl$ , is remarkably efficacious as a bleaching agent for almost any bleaching purpose where hypochlorous acids, hypochlorites, or 25 peroxygen compounds are at present employed.

Tertiary butyl hypochlorite is a pale yellow liquid which is exceedingly stable if kept out of bright light. It is relatively insoluble in water and soluble in various organic solvents such as 30 the chlorinated hydrocarbon solvents, e. g. trichlorethylene, methylene chloride, carbon tetrachloride, perchlorethylene etc., the hydrocarbon solvents such as naphtha, and other petroleum fractions, and in alcohols such as methanol and 35 ethanol. It boils at about 80° C. at atmospheric pressure. While it will quite decompose when stored for some time in the bright sunlight, it is stable in diffused light and exceedingly stable when kept in the dark.

In view of the insolubility of tertiary butyl hypochlorite in water, it has been found most advantageous to dissolve the bleaching agent in an organic solvent and apply it to the material to be bleached dissolved in that solvent. Thus, in 40 the bleaching of cotton or other textile fibers or fabrics it may be dissolved in a chlorinated hydrocarbon solvent such as trichlorethylene, carbon tetrachloride, perchlorethylene or methylene chloride and applied in that solvent to the fabric 45 to be bleached. Similarly, it may be dissolved in any of the hydrocarbons such as benzene or petroleum fractions, or in an alcohol.

When utilizing tertiary butyl hypochlorite for the bleaching or deodorizing of butter, it is merely 50 necessary to introduce a small amount of this

bleaching agent into the butter, thoroughly emulsifying it therein. Similarly, for the bleaching of fats or waxes the tertiary butyl hypochlorite may ordinarily be thoroughly interspersed throughout the solid material to be bleached and 5 need not be applied thereto by means of a solvent. Since some dark-colored materials which are normally bleached commercially will dissolve tertiary butyl hypochlorite it is only necessary in bleaching these materials to introduce a small 10 amount of organic hypochlorite and secure thorough solution therein by agitation.

As an example of the preparation and use of my novel and improved bleaching agent, the following may be given: 15

*Example*

A quantity of tertiary butyl hypochlorite was prepared by adding one mole of tertiary butyl alcohol to a strong solution of caustic soda containing 20 2 moles of NaOH. Sufficient water was added to form a homogeneous mass. Chlorine gas was then passed through the solution, ice water being applied to the reaction vessel in order that the reaction mixture might be maintained 25 at a relatively low temperature.

A yellow mobile layer which was insoluble in the solution separated. This constituted tertiary butyl hypochlorite and it was secured in substantially quantitative yields. The yellow liquid was 30 then removed from the aqueous residue and dried by rapid passage over fused calcium chloride. It was of pale yellow color and possessed a characteristic odor. Its vapor had an irritating effect upon the eyes and mucous membrane of the 35 nose.

Solutions of 2.5% concentration of this compound in each of the following organic solvents were prepared: trichlorethylene, methylene chloride, carbon tetrachloride, naphtha, and 40 ethanol. These solutions were applied to dark-colored cotton materials. Even at room temperature substantial bleaching was apparent, which was increased by elevation of the temperature to 160° F. Waxes and oils present on the 45 cotton were also removed. The resulting product did not experience that objectionable damage which is frequently observed in cotton which has been bleached by application of hypochlorites.

It should be understood that my invention is 50 not to be restricted to precise or exact amounts of the active agent, as the amount of tertiary butyl hypochlorite to be applied in any one instance will depend upon the character of the material being bleached or deodorized and the 55

nature and extent of dark-colored substances present. Various changes may be made in the mode of application of my improved bleaching agent, which may also be used for bleaching materials other than those specified above as illustrative. The invention is not to be restricted to precise numerical amounts, to treatment of specified fabrics or foodstuffs, or to the utilization of the tertiary butyl hypochlorite as bleaching agent only when dissolved in a solvent therefor, but is to be construed in accordance with the appended claims.

I claim:

1. A process of bleaching dark-colored materials which comprises contacting said materials with tertiary butyl hypochlorite.
2. A process of bleaching textile fabrics which comprises contacting said fabrics with tertiary butyl hypochlorite.
3. A process of bleaching textile fabrics which comprises contacting said fabrics with a solution comprising tertiary butyl hypochlorite dissolved in an organic solvent.

PAUL J. CARLISLE.